# EUROPEAN PATENT SPECIFICATION

(11) **EP 0 041 851 B1**
(45) Date of publication and mention of the grant of the patent: **21.03.1984**
(21) Application number: 81302518.6
(22) Date of filing: 05.06.1981
(51) Int. Cl.: C10M 1/08

(54) **Lubricant composition with stabilized metal detergent additive and friction reducing ester component**
Schmiermittelzusammensetzung mit stabilisiertem Metalldetergenzzusatz und mit einer reibungsreduzierenden Esterkomponente
Composition lubrifiante contenant un additif détergent comprenant un métal stabilisé, et un composé d'ester réduisant le frottement

(30) Priority: 09.06.1980 US 157225
(43) Date of publication of application: 16.12.1981
(73) Proprietor: EXXON RESEARCH AND ENGINEERING COMPANY, Florham Park, New Jersey 07932-0390 (US)
(72) Inventor: Rehrer, David Henry, Westfield New Jersey (US)
(74) Representative: Bawden, Peter Charles

## Description

This invention relates to oil compositions which contain both an overbased metal detergent additive and a glycol ester friction modifier. More particularly, this invention relates to a method for formulating such compositions wherein the formation of haze and sediment due to the incompatibility of these additives is overcome.

Lubricating oil compositions containing metal detergent additives being either the normal or basic (overbased) magnesium or calcium sulfurized phenates or sulfonates are well known in the art and are employed in various motor oil formulations. Formulating these metal detergent additives with other ingredients in a finished lubricating oil blend has been known to create compatibility problems, specifically the formation of sediment, separation of phases, visible precipitation or haze and similar problems which are evidence of incompatibility or unwanted interaction of components.

Resolution of this problem through techniques known in the art is represented by U.S. Patent 3,714,042, issued January 30, 1973 to Greenough, which discloses the treatment of overbased complexes with a high molecular weight aliphatic carboxylic acid or anhydride at elevated temperatures. U.S. Patent 3,965,017, issued to Burnop et al discloses stabilization through addition of small proportions of a monocarboxylic acid, anhydride or salt or the reaction product of a hydrocarbon with P₂S₅ and a glycol or ether alcohol.

Lubricant compositions containing the polycarboxylic acid-glycol ester friction modifier additive used in the compositions of the present invention are disclosed in U.S. Patent 4,105,571 issued to Shaub et al.

The present invention is concerned with resolution of the specific problem of incompatibility encountered when lubricating oil formulations are prepared which contain both a metal or overbased metal sulfonate or a sulfurized phenate detergent additive, particularly where the metal is calcium or magnesium, and small proportions of a glycol-polycarboxylic acid ester friction reducing additive.

In accordance with the present invention, there is provided a lubricating oil composition having a reduced tendency toward sediment formation, which comprises a glycol-polycarboxylic acid ester friction reducing additive and a metal detergent additive being a metal or overbased metal sulfonate or sulfurized phenate, which composition is prepared by a process comprising the steps of :
(a) providing a lubricating oil mixture containing a lubricating oil base stock containing about 0.1 to 10 percent by weight of a metal or overbased metal sulfonate or sulfurized phenate detergent additive ;
(b) treating said mixture by reacting said metal detergent additive with from about 50 to 100 percent by weight, based upon the weight of the metal detergent additive, with either (i) a phosphosulfurized polyisobutylene or (ii) a polyisobutenyl succinic anhydride at temperatures of from about 55 °C to about 225 °C for a period of from about 2 to 30 hours ; and
(c) thereafter, adding to said treated mixture about 0.01 to about 2.0 percent by weight, based on the total weight of the composition, of said glycol ester friction modifier additive, whereby said composition exhibits a reduced tendency toward phase separation or sediment or haze formation.

The metal detergent additives used in the present invention are those metal or overbased metal sulfonate or sulfurized phenate oil-soluble additives which are well known in the art. The metal sulfonates are obtained from sulfonic acids derived from sulfonating natural or synthetic hydrocarbons, such as by treating oil base stocks with concentrated or fuming sulfuric acid or by sulfonating alkylated aromatic hydrocarbons. The hydrocarbyl sulfonate of these metal detergent additives is derived from petroleum sulfonates and includes alkyl, alkylaryl and aryl sulfonates and mixtures thereof having a molecular weight of from about 300 to 1,000, such as barium nonylbenzene sulfonate, magnesium dodecylbenzene sulfonate and the like. The sulfonates are usually the alkaline earth metal sulfonates, usually calcium, barium, or magnesium, but can also be alkali metal sulfonates, such as sodium sulfonates. Overbased sulfonates are those which contain metal base in excess that is required for simple neutralization. In preparing such overbased materials, the sulfonic acid is typically reacted with an excess of metal base and the excess base is usually neutralized with an acidic gas, such as carbon dioxide. Such overbased sulfonates have a total base number (ASTM-D-664) of about 50 to 500.

The sulfurized phenates are the metal salts of sulfurized alkyl phenols, which contain about 2 to 14 percent by weight sulfur based on the weight of the sulfurized alkyl phenols. Such materials are well known in the art and are derived from alkylated phenols, wherein the alkyl is C₅-C₄₀, such as t-amyl phenol, t-octyl phenol, nonylphenol, di-t-octyl phenol and phenols alkylated with suitable polymers of up to 40 carbon atoms obtained from propylene, butylene, amylenes or mixtures thereof. The sulfurized phenols are prepared by well-known methods, for example, by reacting the alkylated phenol with sulfur monochloride, sulfur dichloride or elemental sulfur.

The metals employed for providing the phenate salts are typically alkali metal, alkaline earth metal or magnesium, principally calcium or magnesium. Overbased phenates are prepared by the process comprising reacting the phenol with excess base and the excess is neutralized with carbon dioxide. Typical overbased metal sulfurized phenates will have a total base number (ASTM-D-664) of about 50 to 100.

The treatment step of the present invention generally comprises incorporating the metal detergent additive into a lubricating oil and conducting a reaction for about 2 to 30 hours at temperatures of from about 55 °C to 225 °C with either a phosphosulfurized polyisobutylene or with a polyisobutenyl succinic anhydride, and 25-100 percent, preferably 50-100, percent by weight of these materials are used based upon the weight of the metal detergent additive present.

When employing a phosphosulfurized polyisobutylene, it is preferable in most cases to conduct the treatment step of the present invention at relatively higher temperatures and longer periods of time. Thus, the preferred treatment conditions for P₂S₅-polyisobutylene treatment are temperatures of about 100 °C to 200 °C and a treatment period of about 10 to 25 hours, particularly when the metal additive is an overbased calcium or magnesium sulfurized phenate.

When the polyisobutenyl succinic anhydride is employed, preferred conditions of treatment in accordance with this invention are temperatures of about 60 °C to 85 °C for about 2 to 7 hours.

Phosphosulfurized polyisobutylenes useful in the present invention are prepared by methods well known in the art comprising the reaction of sulfides of phosphorous with polyisobutylene at elevated temperatures. While P₂S₅ is preferred, P₂S₃, P₄S₃ and P₄S₅ are also useful as well as mixtures thereof, as well as mixtures of elemental phosphorous and sulfur. The reaction is carred out at about 90 °C to 315 °C, preferably 150 °C, to 290 °C, using about 1 to 5 molar proportions of polyisobutylene to 1 molar proportion of phosphorous sulfide. The reaction is usually continued until the maximum amount of sulfur or phosphorous sulfide has been added but this is not essential to provide a useful product. Typical reaction times are about 2 to 10 hours. Generally, the polyisobutylenes have a molecular weight of about 500 to 25,000, preferably 800 to 2,000. Particularly useful are polyisobutylene of 700 to 1,500 molecular weight reacted with about 10 to 15 percent by weight of P₂S₅.

The polyisobutenyl succinic anhydrides useful herein for treating the metal detergent additives are also known and are disclosed in the number of references, such as U.S. Patent 3,288,714, issued to Osuch. These are oil-soluble materials, which have desirable additive properties themselves, principally as dispersants, prepared by reacting maleic anhydride with a polyisobutylene polymer having a molecular weight of about 500 to 2,000. Particularly preferred for use as treating agents in the present invention are those polyisobutenyl succinic anhydrides wherein the polyisobutenyl group has a number average molecular weight of about 700 to 1,500.

The lubricating oil base stock employed herein generally comprises a hydrocarbon mineral oil of lubricating viscosity including paraffinic, naphthenic and aromatic oils preferably a mineral paraffinic oil having a viscosity of about 20 to 100 mm²/s min. 37.8 °C and blends of such mineral paraffinic oils. Synthetic oils may be used provided the conditions of treatment do not adversely affect such synthetic oils by causing an unwanted side reaction.

The finished formulation then may be prepared by incorporating into the treated composition the friction reducing polycarboxylic acid glycol ester which is employed in amounts of about 0.01 to 2.0 percent preferably 0.05 to 0.3 percent by weight, typically, 0.1 to 0.3 percent by weight based upon the total weight of the composition being used. The friction reducing esters are described in more detail hereinbelow.

The friction reducing esters are generally derived from the esterification of a polycarboxylic acid with a glycol and may be partial esters or diesters of the formulas : wherein R is the hydrocarbon radical of the acid and R' and R" is either the hydrocarbon radical of an alkane diol or the oxyalkylene radical from an oxa-alkane diol as defined hereinbelow. The polycarboxylic acid may be an aliphatic saturated or unsaturated acid and will generally have a total of about 24 to 90, preferably about 24 to 60, carbon atoms and about 2 to 3, preferably about 2, carboxylic acid groups with a least about 9 carbon atoms, preferably about 12 to 42, especially 16 to 22 carbon atoms between the carboxyclic acid groups. Generally about 1-3 moles of glycol, preferably 1-2 moles of glycol, is used per mole of acid to provide'either a complete or partial ester. Esters within the foregoing formula can also be prepared by reaction of the acid with 1 mole or more of ethylene oxide.

Also, esters can be obtained by esterifying a dicarboxylic acid or mixture of such acids with a diol or mixture of diols, R would then be the hydrocarbon radical of the dicarboxylic acid and R' and R" would be the hydrocarbon radical associated with the diols or diols.

Especially preferred are the dimer acid ester friction reducing esters. The term dimer acid used herein is meant to refer to those substituted cyclohexene dicarboxylic acids formed by a Dieis-Aider-type reaction which is a thermal condensation of Cₗ₈-C₂₂ unsaturated fatty acids, such as tall oil fatty acids which typically contain about 85 to 90 percent oleic or linoleic acids. Such dimer acids typically contain about 36 carbon atoms. The dimer acid structure can be generalized as follows : with two of the R groups being carboxyl groups and two being hydrocarbon groups depending upon how the condensation of the carboxylic acid has occurred. The carboxyl groups can be -(CH₂)_{B}COOH ; ―CH=CH(CH₂)₇GOOH ; ―(CH₂)₇COOH ; ―CH₂CH=CH(CH₂)₇COOH ; ―CH=CH(CH₂)₇COOH and the hydrocarbon terminating group can be represented by: CH₃(CH₂)₄― , CH₃(CH₂)₅― ; CH₃(CH₂)₇ ; ―CH₃(CH₂)₄CH=CH― ; CH₃(CH₂)₄CH=CH CH₂―; CH₃(CH₂)₄CH=CH CH₂―; and the like. The dimer of linoleic acid which is the preferred embodiment can be expressed in the following formula :

Also the term dimer acid as used herin necessarily includes products containing up to about 24 percent by weight trimer, but more typically about 10 percent by weight trimer since, as is well Known in the art, the dimerization reaction provides a product containing a trimer acid having molecular weight of about three times the molecular weight of the starting fatty acid.

The polycarboxylic acids or dimer acids noted above are esterified with a glycol, the glycol being an alkane diol or oxa-alkane diol represented by the formula HO(RCHCH₂0)ₓH wherein R is H or CH₃ and x is about 2 to 100, preferably 2 to 25, with ethylene glycol and diethylene glycol particularly preferred. A preferred embodiment is formation of the ester with about 1 to 2 moles of glycol per mole of dimer acid or polycarboxylic acid, such as the ester of diethylene glycol with dimerized linoleic acid.

Numerous other additives will of course normally be included in a finished lubricating oil composition such as detergents and dispersants, oxidation and rust inhibitors, viscosity index improvers, pour depressants, anti-wear agents and the like and these may be added prior to or subsequent to the addition of the friction reducing ester component.

### Examples

Formulations were prepared which demonstrated the incompatibility of the metal detergent additive with a dimer acid ester friction modifier which in each formulation was diethylene glycol ester of dimerized linoleic acid. In each formulation set forth in Table I, the composition was cloudy with visible separation of phases after standing for several days both at room temperature and at 65 °C. The base oil in each case was Solvent 150 Neutral oil, a mineral paraffinic oil having a viscosity of 31 mm²/s min. at 37.8 °C.

In each formulation of Table I, in the absence of the friction modifier additive the formulations were clear with no evidence of instability after storage for equivalent periods of time under the same conditions. Total base numbers reported are according to ASTM-D-664.
(1) Overbased calcium sulfurized dodecyl phenate sulfide having a total base number of 250.
(2) Overbased magnesium sulfurized nonylphenate, nonylphenol sulfide having a total base number of 250.
(3) Overbased magnesium alkyl sulfonate having a total base number of 395.
(4) Overbased calcium alkyl sulfonate having a total base number of 300.
(5) Calcium sulfurized dodecyl phenate having a total base number of 135.

A number of stabilized formulations were prepared by first treating an oil concentrate containing 20-30 wt. percent of the metal detergent additive with a P₂S₅-polyisobutylene (mol. wt. 780) and then blending with the base oil and friction modifier to provide the finished formulation. These are set forth in Table II which includes the various treatment times and temperatures used ; all formulations were clear with no evidence of instability upon standing for 1 month at room temperature and 1 month at 65 °C. The metal additives and friction modifier are the same as those reported in Table I.

Similarly, metal detergent additives were treated with two types of polyisobutenyl succinic anhydrides ; formulations A & B used Mn = 1,000 and Sap No. 112 and formulations C & D used Mn = 1,300 and Sap. No. 103 under varying conditions of time and temperature and, thereafter, the treated materials were blended into the formulations reported in Table III each of which remained clear upon storage for 1 month at room temperature and 1 month at 65 °C with no instability apparent. Again, the base oil, additives and friction modifiers are those identified in the prior examples.

Instead of carrying out the treatment of the detergent additive in a lubricating oil, the same results are obtained by carrying out the treatment in a lubricating oil concentrate wherein said detergent additive is present in amounts of 20 to 50 wt. percent, based on the total oil composition, the base oil comprising 50 to 80 percent of the composition, or a portion of the oil may be replaced by other additives, such as viscosity index improver, pour depressants, dispersants, etc. Thus, 0.1 to 50 wt. percent of the detergent additive admixed with the oil can be used in the reaction with said phosphosulfurized polyisobutylene or anhydride reactants.

## Claims

1. An oil composition comprising a lubricating oil base stock, a polycarboxylic acid glycol ester friction modifier additive and a metal or overbased metal sulfonate or sulfurized phenate detergent additive which composition is prepared by a process comprising the steps of :
a) providing a mixture containing a lubricating oil base stock and 0.1 to 50 percent by weight of the metal detergent additive ;
b) treating said mixture by reacting it with 25 to 100 percent by weight, based on the weight of the metal detergent additive, with either a phosphosulfurized polyisobutylene or a polyisobutenyl succinic anhydride at temperatures of from 55° to 225 °C for 2 to 30 hours, and
c) thereafter adding to said treated mixture 0.01 to 2.0 percent by weight, based on the total weight of the composition, of the glycol ester friction modifier additive, whereby said composition exhibits a reduced tendency toward sediment formation or phase separation.

2. The composition of claim 1 wherein the metal detergent additive is an overbased calcium or magnesium sulfonate.

3. A composition of claim 1 wherein the metal detergent additive is an overbased calcium or magnesium sulfurized phenate.

4. The composition of claims 1 or 2 wherein said treatment step is conducted with a polyisobutenyl succinic anhydride wherein the polyisobutenyl group has a molecular weight of from 700 to 1,500.

5. The composition of claims 1-4 wherein the friction modifier is the diethylene glycol ester of the dimer acid of linoleic acid.

6. The composition of claim 5 wherein the concentration of said glycol ester is from 0.05 to 0.3 weight percent.

7. The composition of claims 1-3 wherein said treatment step is conducted with a polyisobutylene of 700 to 1500 molecular weight phosphosulfurized with P_{Z}S_{S}.

8. The composition of claim 7 wherein said treatment step is conducted at a temperature of from 100 °C to 200 °C for a period of about 10 hours to 25 hours.

9. The composition of claim 4 wherein the treatment is conducted at a temperature of from 60° to 85 °C for 2 to 7 hours.

10. The composition of claims 1-9 wherein said treatment is carried out on a mixture containing said lubricating oil base stock and 0.1 to 10 percent by weight of said metal detergent additive, using 50 to 100 percent by weight, based on the weight of said metal detergent additive, of said phosphosulfurized polyisobutylene or of said anhydride.

## Patentansprüche

1. Ölzusammensetzung, die ein Schmieröl als Basis, ein Polycarbonsäureglykolester-Reibungsmodifiziermitteladditiv und ein Metall- oder überbasisches Metallsulfonat- oder sulforiertes-phenat-Tensidadditiv enthält, erhältlich ist nach einem Verfahren mit den folgenden Verfahrensstufen :
a) Zurverfügungstellung einer Mischung, die ein Schmieröl als Basis und 0,1 bis 50 Gew.% des Metall-Tensidadditivs enthält ;
b) Behandlung dieser Mischung durch Umsetzung mit, bezogen auf das Gewicht des Metall-Tensidadditivs, 25 bis 100 Gew.% entweder eines phosphorsulforierten Polyisobutylens oder eines Polyisobutenylbernsteinsäureanhydrids bei Temperaturen von 55 bis 225 °C über einen Zeitraum vom 2 bis 30 Stunden ; und
c) anschließender Zusatz von bezogen auf das Gesamtgewicht der Zusammenstzung 0,01 bis 2,0 Gew.% des Glykolester-Reibungsmodifizierungsmitteladditivs zu der behandelten Mischung, und eine verringerte Neigung zur Sedimentbildung oder Phasentrennung zeigt.

2. Zusammensetzung nach Anspruch 1, dadurch gekennzeichnet, daß das Metall-Tensidadditiv ein überbasisches Calcium- oder Magnesiumsulfonat ist.

3. Zusammensetzung nach Anspruch 1, dadurch gekennzeichnet, daß das Metall-Tensidadditiv ein überbasisches, sulforiertes Calcium- oder Magnesiumphenat ist.

4. Zusammensetzung nach Anspruch 1 oder 2, dadurch gekennzeichnet, daß die Behandlungsstufe mit einem Polyisobutenylbernsteinsäureanhydrid durchgeführt wird, wobei die Polyisobutenylgruppe ein Molekulargevicht von 700 bis 1 500 besitzt.

5. Zusammensetzung nach Anspruch 1 bis 4, dadurch gekennzeichnet, daß das Reibungsmodifiziermittel der Diethylenglykolester der dimeren Säure von Linolsäure ist.

6. Zusammensetzung nach Anspruch 5, dadurch gekennzeichnet, daß die Konzentration des Glykolesters 0,05 bis 0,3 Gew.% beträgt.

7. Zusammensetzung nach Anspruch 1 bis 3, dadurch gekennzeichnet, daß die Behandlungsstufe durchgeführt wird mit einem Polyisobutylen mit einem Molekulargewicht von 700 bis 1 500, das mit P₂S₅ phosphosulfuriert worden ist.

8. Zusammenstzung nach Anspruch 7, dadurch gekennzeichnet, daß die Behandlungsstufe bei einer Temperatur von 100 bis 200 °C über einen Zeitraum von etwa 10 bis 25 Stunden durchgeführt wird.

9. Zusammensetzung nach Anspruch 4, dadurch gekennzeichnet, daß die Behandlungsstufe bei einer Temperatur von 60 bis 85 °C über 2 bis 7 Stunden durchgeführt wird.

10. Zusammensetzung nach den Ansprüchen 1 bis 9, dadurch gekennzeichnet, daß die Behandlung unter Verwendung von, bezogen auf das Gewicht des Metall-Tensidadditivs, 50 bis 100 Gew.% des phosphosulfurierten Polyisobutylens oder des Anhydrids mit einer Mischung durchgeführt wird, die das als Basis dienende Schmieröl und 0,1 bis 10 Gew.% des Metall-Tensidadditivs enthält.

## Revendications

1. Composition d'huile comprenant une huile lubrifiante de base, un ester de glycol d'acide polycarboxylique comme additif modificateur de friction et un sulfonate ou un phénate sulfuré de métal ou de métàl rendu surbasique comme additif détergent, cette composition étant obtenue par un procédé comprenant les étapes suivantes :
a) préparation d'un mélange contenant une huile lubrifiante de base et 0,1 à 50 % en poids de l'additif détergent métallique ;
b) traitement dudit mélange par sa réaction avec 25 à 100 % en poids, sur la base du poids de l'additif détergent métallique, d'un polyisobutylène phosphosulfuré ou d'un anhydride polyisobuténylsuccinique à des températures de 55 à 225 °C pendant 2 à 30 heures, puis
c) addition audit mélange traité de 0,01 à 2,0% en poids, sur la base du poids total de la composition, d'un ester glycolique additif modificateur de friction, ladite composition présentant une tendance réduite à la formation d'un sédiment ou à la séparation en phases.

2. Composition suivant la revendication 1, dans laquelle l'additif détergent métallique est un sulfonate de calcium ou de magnésium rendu surbasique.

3. Composition suivant la revendication 1, dans laquelle l'additif détergent métallique est un phénate sulfuré de calcium ou de magnésium rendu surbasique.

4. Composition suivant la revendication 1 ou 2, dans laquelle ladite étape de traitement est conduite avec un anhydride polyisobuténylsuccinique dont le groupe polyisobutényle a un poids moléculaire de 700 à 1 500.

5. Composition suivant les revendications 1-4, dans laquelle le modificateur de friction est l'ester de diéthylène-glycol du dimère de l'acide linoléique.

6. Composition suivant la revendication 5, dans laquelle la concentration dudit ester de glycol va de 0,05 à 0,3 % en poids.

7. Composition suivant les revendications 1-3, dans laquelle ladite étape de traitement est conduite avec un polyisobutylène de poids moléculaire égal à 700-1 500, phosphosulfuré avec P₂S_{5'}

8. Composition suivant la revendication 7, dans laquelle ladite étape de traitement est conduite à une température de 100 à 200 °C pendant une période d'environ 10 à 25 heures.

9. Composition suivant la revendication 4, dans laquelle le traitement est conduit à une température de 60 à 85 °C pendant 2 à 7 heures.

10. Composition suivant les revendications 1-9, dans laquelle ledit traitement est conduit sur un mélange contenant ladite huile lubrifiante de base et 0,1 à 10 % en poids dudit additif détergent métallique en utilisant 50 à 100% en poids, sur la base du poids dudit additif détergent métallique, dudit polyisobutylène phosphosulfuré ou dudit anhydride.
